# EUROPEAN PATENT SPECIFICATION

(11) **EP 1 324 888 B1**
(45) Date of publication and mention of the grant of the patent: **19.05.2004**
(21) Application number: 00962161.6
(22) Date of filing: 26.09.2000
(51) Int. Cl.: B44C 5/04, B44F 7/00

(54) **METHOD OF PRODUCING A DECOR ON A GLASS WALL OR FLOOR TILE**
VERFAHREN ZUR HERSTELLUNG EINES DEKORS AUF EINER WAND- ODER BODENFLIESE
PROCEDE DE PRODUCTION DE DECOR SUR UNE PLAQUE DE VERRE OU SUR DU CARRELAGE

(43) Date of publication of application: 09.07.2003
(73) Proprietor: Sorm, Michal, 190 00 Praha 9 (CZ)
(72) Inventor: Sorm, Michal, 190 00 Praha 9 (CZ)
(74) Representative: Patentservis Praha a.s.
(86) International application number: PCT/CZ2000/000073
(87) International publication number: WO 2002/026509

(56) References cited:
- EP-A- 0 411 152
- EP-A- 0 974 714
- DE-U- 9 402 364
- GB-A- 913 995
- GB-A- 2 245 223

## Description

### Field of the Invention

The present invention relates to a glass wall or floor tile, particularly to a method of producing a decor on such tile to bring about an image exhibiting special light effects.

### Background of the Invention

It is known in the art to produce patterns or images with special light effects, so as for example by reflection of light from matt surfaces, from glossy surfaces or from objects within a transparent material when light passes through it or by passage of light through a system of transparent layers and optical layers, when the resultant pattern or image is formed which pattern or image depends on the illumination intensity or on the view angle.

In case of the glass plates used to decorate buildings, the decor of such plates is brought about by printing or by spraying ink on such plate, which ink is then fired to obtain a permanent sun resistant colour decor. Also, it is known to provide the plates with a printed colour decor made of an inorganic material with subsequent tempering, whereby, a decor exhibiting intensive decorative effect is obtained, which decor is abrasion resistant, yields fast colour and is suitable to decorate both the interior and the exterior.

Also, it is known to decorate glass plates by printing with ink on glass, which ink is then fired and then by sticking glass fragments on the decorated surface and the resultant system is then sintered and annealed to yield a rough surface which surface is then coated with a binder which binder is then left to set.

Also, it is known to insert melted metal pattern elements between two endless bands of glass, which bands are formed by rolling.

In case of forming images by means of a system of layers, such layers are appropriately grouped and connected by suitable binders or adhesives.

Another method of producing decor consists in forming glass between rollers, which glass was previously softened by melting, whereby, one of the rollers is provided with convex or concave patterns, which patterns are transferred onto the surface of glass, and the glass is then cooled. Thereby, plates suitable for decoration of kitchens, bathrooms or buildings are obtained. Also, it is known to produce decors by connecting rasters of images and/or signs, for example of characters, which rasters are put on each other, whereby, the rasters are formed by films provided with systems of printed elements.
However, at a given configuration of the optical environment the above specified solutions do not allow to create exactly defined patterns simply, at an acceptable price, in the required quality and in a number of variations on at least partially transparent and hard materials, for example on glass.

### Summary of the Invention

The above mentioned drawbacks are removed by a method of producing decor on a glass wall or floor tile used to yield an image provided with special light effects according to the present invention which method consists in that on specified opposite surfaces of the front and the back sides of a glass plate a system of decorative elements of decreased transparency or opacity is produced, which system forms a decor in the shape of at least one segment composed of arranged transparent signs and slots on each side of the plate, whereby the decorative elements of at least the front side are formed by ink and/or by hot rolling glass and/or by grinding glass, whereupon, the used decoration ink is further treated in accordance with the kind of the decoration material to obtain specific mechanical properties, and finally, final formatting and calibrating of the plate is carried out.

According to one preferable embodiment of this invention the decor of the plate back side is produced by fixing a film provided with a system of printed decoration elements to the back side of the plate.

According to another preferable embodiment of the present invention the system of decorative elements of decreased transparency or opacity is determined by finding out light effect deviations of the basic design of the layout of said elements in comparison to the desired resultant light effect and by carrying out a correction of deviations by changing at least one of the characteristics of at least one segment on one of the plate sides, whereby, said characteristics comprise number, size and density of the transparent signs and slots, segment orientation and colour alternative.

Preferably, the decorative elements are produced by applying heat fireable ink, which ink is applied by printing, spraying, putting ink into sunken areas and by using a decal. Glass ink, ceramic ink, metal ink or enamel can be used as the fireable ink.

If the decorative elements are produced by rolling or grinding of the glass surface, it is preferable to fill the sunken areas with heat fireable ink.

According to another preferable embodiment of the method according to this invention, the decorative elements are produced by using non-heat-fireable inks, for example those based on resins, enamels, UV-light hardenable inks or chemically crosslinkable inks.

Also, it is preferable to modify the used decorative ink further by firing or by drying or hardening it to obtain specific mechanical properties that are in accordance with the kind of the decorative material.

By the method according to the present invention exactly delimited patterns of a superior quality are produced simply and cost effectively so that they are determined for broad scope of applications. If the fireable inks are used, glass plates exhibiting special mechanical characteristics are obtained, which properties are a prerequisite of their use as the wall or floor plates. According to the method of this invention, patterns and the colour designs can be produced quickly and simply in a number of variations.

### Detailed Description of the Invention

A glass planar transparent or slightly coloured plate having dimensions up to 4 m x 5 m and thickness 1 to 25 mm is used as the starting blank plate.

At first, it is determined what opposite surface areas of the front and back sides and in what way will use a decor to yield light effects. Such selected surface areas are then decorated according to the respective project by applying a system of decorative elements exhibiting decreased transparency or opacity, whereby, such elements are grouped so as to produce a decor in the form of at least one segment of the arranged, transparent signs and slots on each side of the plate. The slots can also be continuously interconnected with signs, whereby, the segment always has one prevailing orientation or, to put it differently, one direction of slots or signs.

Preferably, the appearance of the resultant light effect is checked and eventually the original design of decorative elements layout is modified to obtain the optimal effect.

It is carried out in such a way that the light effect differences of the basic design of a system of the decreased transparency or opaque decorative elements in comparison to the original project are determined and the respective corrections of differences are carried out by modifying at least one of the characteristics of at least one segment.

To make a correction, changes of individual segment(s) characteristics of only one side of the plate are tested one after the other. The respective characteristics are the slot size, their length or width, further then the angular position of the segment(s), change in orientation of the segment(s), then the number and density of slots in the segment (s) or the size and density of signs and then colour combinations. The corrections can be carried out in a laboratory by means of a film, glass, etc., or directly during a visual evaluation by adjusting the printing machine producing the decor, i.e. by turning the machine into such position when the light effects are produced. For example, if a greater difference in the number of similarly oriented slots in the segments of both plate sides are applied, the light effect is increased. Also, in case of a greater difference in angular position of the segments, the light effect is increased. By a mutual combination of both factors the optimal effect can be obtained. In case, smaller size of the transparent slots and signs is chosen, decomposition and diffusion of light plays a greater role.

After final design of the decor, the method for producing decorative elements on plate sides is determined. The elements can be produced by applying ink, by rolling or by grinding or by combinations of said methods or by means of applying a printed film.

It is possible to produce a decor by the same method on both sides of the plate or a different method on both sides. For example, ink is used on the front plate side and a printed film is applied on the rear plate side, so as it will be described in greater detail below.

If a high hardness, abrasive resistance and chemical stability are required, fireable inks are used to produce the decor. A cheaper production combined but with lower durability in use is obtained if non-fireable inks are used.

### The ink can be applied by one of the following methods:

A blank glass plate, is formatted to the desired dimensions, e.g. by cutting, grinding, etc., and the plate is then provided with ink print by screen or rotary printing.

Instead of screen printing, flexography can be used, whereby, the ink is applied on the relief on the surface of a flexible roller and the ink is then transferred to the glass surface. It is necessary to take into account that because of roller flexibility the decorative signs may not be entirely precisely demarked.

The ink can be applied on the blank plate also by spraying using a mask or a masking layer to cause that the ink gets only to the predetermined places for the required decor.

The decorating ink can also be applied on a blank plate by injecting when an programmable injection printer is used to inject the ink on predetermined places to yield the required decor.

Making of decorative elements by ink is a substitution of expensive and for small-series production unsuitable colouring of glass. It is more variable, by providing ink print on both sides the tile becomes coloured. It is preferable to coat at least 30 % of the front side area of the tile with ink.

The ink can also be wiped into the blank plate. A system of decorative elements is ground or hot rolled into the areas of the plate sides (so as it will be specified in detail later). Then, the whole area is coated with ink and wiped with a blade so that the ink remains only in the sunken areas, whereby, the required decor will be formed.

Finally the decorating ink can be transferred to the blank plate by means of a decal. The respective arrangement of segments is applied by transferable ink on a carrier substrate, e.g. a paper, by a screen printing method and the transferable ink is then transferred to the blank plate.

After forming decorative elements, it is proceeded in accordance with the used ink material. This material is either fired using the respective temperature and firing temperature course to obtain minimal or maximal material stress, i.e. the ink is hardened, or the decorative material is left to dry or it is hardened using a source of UV light, eventually, it is hardened chemically.

Also, the front side of the plate can be decorated by hot rolling. This method uses changes in optical boundary and surface transparency in hot rolling. The unrolled part of the plate maintains its original optical characteristics, which characteristics are identical with those of the transparent signs and slots. The rolled part yields optical characteristics that are modified according to the roughness and the depth of the recesses provided. More particularly, a blank plate is rolled at 500 to 800 °C by means of a pressing tool, which tool presses recesses into the glass surface. The recesses have depth 0.001 to 1.0 mm. A system of decorative elements is so formed. Considering that after cooling the recesses exhibit different optical properties in comparrison to the non press treated surrounding area, the optical boundaries and interference can be used to some extent together with the back side decorated by some of the above mentioned methods of decoration by ink. To increase the colour effect, it can be preferable to fill the recesses obtained by pressing using the above mentioned method of putting ink into the recesses.

Further, it is possible to decorate the front side by grinding. Again, recesses are formed in the respective part of the surface so as in the previous case. For the grinding, the standard methods of grinding can be used. To modify optical characteristics of the ground plate parts, it is possible to use the same method as in case of rolling.

The rear plate side can be decorated using substantially the same methods as in the case of the front plate side. In case there are no high demands on hardness, it is possible to use sticking a film on it, which film is provided with a printed system of decorative signs. When the above mentioned methods of the plate front side decoration are used to decorate the back side, or their combination, the respective thermal process can be integrated into one operation, whereby, it can be made more rapid and simple.

When both sides of the plate have been decorated, the final formatting and calibrating of the plate is carried out.

### Industrial Use

The present invention can be used to produce tiles provided with exact and special decor yielding many colour or image combinations by a rapid, easy, cheap and variable method.

## Claims

1. A method of producing decor on a glass wall or floor tile used to yield an image provided with special light effects obtained by passage of light through at least semitransparent plate material with a first surface pattern decor on the face front side and another surface pattern decor on the back rear side different from said first décor and spaced from it, **characterized in that** on specified opposite surfaces of the front and the back sides of a glass plate a system of decorative elements of decreased transparency or opacity is produced, which system forms a décor in the shape of at least one segment composed of arranged transparent signs and slots on each side of the plate, whereby the decorative elements of at least the front side are formed by ink and/or by hot rolling glass and/or by grinding glass, whereupon, the used decoration ink is further treated in accordance with the kind of the decoration material to obtain specific mechanical properties, and finally, final formatting and calibrating of the plate is carried out.

2. A method of Claim 1, **characterised in that** the decor of the plate back side is produced by fixing a film provided with a system of printed decoration elements to the back side of the plate.

3. A method of Claim 1 or Claim 2, **characterised in that** the system of decorative elements of decreased transparency or opacity is determined by finding out light effect deviations of the basic design of the layout of said elements in comparison to the desired resultant light effect and by carrying out a correction of deviations by changing at least one of the characteristics of at least one segment on one of the plate sides, whereby, said characteristics comprise number, size and density of the transparent signs and slots, segment orientation and colour alternative.

4. A method of any of the foregoing Claims, **characterised in that** the decorative elements are produced by applying heat fireable ink, which ink is applied by printing, spraying, putting ink into sunken areas or by using a decal.

5. A method of any of the Claims 1 to 3, **characterised in that** the decorative elements are produced by filling the sunken areas, having been formed by rolling or grinding, with heat fireable ink.

6. A method of any of the Claims 1 to 3, **characterised in that** heat fireable ink is used, preferably glass ink, ceramics ink, metal ink or enamel.

7. A method of any of the Claims 1 to 5, **characterised in that** non-heat-fireable ink, preferably ink based on resins, enamels, UV-light hardenable or chemically crosslinkable inks are used.

8. A method of any of the foregoing Claims, **characterised in that** the used decorative ink is subsequently modified by firing, drying or hardening.

## Patentansprüche

1. Verfahren zur Bildung eines Dekors an einer Glas- oder Fussbodenplatte, das zum Erzielen eines Bilds mit speziellen Lichteffekten bestimmt ist, welche Lichteffekte mit dem Durchgang des Lichts durch ein mindestens semitransparentes Plattenmaterial mit einem ersten Musterdekor an der ersten vorderen Seite und einem zweiten, von dem ersten Musterdekor abweichenden und davon entfernten Musterdekor an der zweiten hinteren Seite erreicht werden, **dadurch gekennzeichnet, dass** an den spezifischen entgegenliegenden Oberflächen der vorderen und hinteren Seiten der Glassplatte ein System von dekorativen Elementen mit verminderter Transparenz oder Undurchsichtigkeit erreicht wird, welches System ein Dekor in der Form mindestens eines Segments bildet, welches Segment aus angeordneten durchsichtigen, mit einer Farbe oder Glastinte und/oder mit dem Glaswarmwalzen und/oder mit dem Glasschleifen erzielten Zeichen und Spalten an jeder Seite der Platte besteht, wobei die Dekorfarbe oder -tinte weiter nach der Art des Dekorationsmaterials zum Erreichen von spezifischen mechanischen Eigenschaften angepasst und endlich ein Formieren und eine Kalibrierung der Platte durchgeführt wird.

2. Verfahren nach Anspruch 1, **dadurch gekennzeichnet, dass** das Dekor an der hinteren Seite der Platte durch das Anbringen einer Folie mit einem System von gedruckten Dekorationselementen an die hintere Seite der Platte hergestellt wird.

3. Verfahren nach Anspruch 1 oder 2, **dadurch gekennzeichnet, dass** das System von dekorativen Elementen mit verminderter Transparenz oder Undurchsichtigkeit durch das Auffinden von Abweichungen der Lichteffekte der Grundmusteranordnung dieser Elemente im Vergleich mit dem verlangten Endlichteffekt und durch das Ausführen von Korrektionen der Abweichungen durch die Änderung von mindestens einer Charakteristik mindestens eines Segments an einer Seite der Platte bestimmt wird, wobei diese Charakteristiken die Anzahl, die Abmessungen und die Dichte der transparenten Zeichen und Spalten, die Orientierung der Segmente und deren Farbalternativen enthalten.

4. Verfahren nach einem der vorhergehenden Ansprüche, **dadurch gekennzeichnet, dass** die dekorativen Elemente durch das Verwenden von aufbrennbaren Farben oder Tinten hergestellt werden, welche Farbe oder Tinte durch das Drucken, Spritzen, Anbringen der Farbe oder Tinte in vertiefte Bereiche der Platte oder durch die Verwendung einer Aufbrennetikette erreicht wird.

5. Verfahren nach einem der Ansprüche 1 bis 3, **dadurch gekennzeichnet, dass** die dekorativen Elemente durch das Ausfüllen der vertieften, mit Walzen oder Schleifen hergestellten Bereichen der Platte mit einer aufbrennbaren Farbe oder Tinte erreicht werden.

6. Verfahren nach einem der Ansprüche 1 bis 3, **dadurch gekennzeichnet, dass** eine aufbrennbare Farbe oder Tinte, insbesondere Glasstinte, Keramiktinte, Metalltinte oder Emaille verwendet wird.

7. Verfahren nach einem der Ansprüche 1 bis 5, **dadurch gekennzeichnet, dass** eine unaufbrennbare Farbe oder Tinte, insbesondere eine Farbe oder Tinte auf der Basis von Harz, von Emaillen, von mit UV-Strahlen gehärteten oder chemisch vernetzten Farben verwendet wird.

8. Verfahren nach einem der vorhergehenden Ansprüche, **dadurch gekennzeichnet, dass** die verwendete dekorative Farbe oder Tinte mit Aufbrennen, Trocknen oder Aushärten anschliessend modifiziert wird.

## Revendications

1. Procédé de production d'un décor d'une plaque en verre destinée à la création des revêtements et carrelages, ledit décor servant à l'engendrement d'un image avec des effets lumineux particuliers dûs au passage de la lumière par la matière du moins partiellement transparente de la plaque comportant le premier décor plan à dessins sur sa face et le deuxième décor plan à dessins sur son côté derrière distinct dudit premier décor et distant de lui, **caractérisé en ce que** les surfaces prévues des côtés opposés de la plaque sont munis d'un système des éléments décoratifs opaques ou de la transparence réduite formant ainsi le décor caractéristique sous forme du moins d'un segment des fentes et des caractères arrangés, lesdits éléments décoratifs sont produits au moins sur la face de la plaque par le colorant et/ou par la lamination à chaud et/ou par le doucissage du verre, le colorant étant traité selon la nature de la matière décorative en vue de l'obtention des propriétés mécaniques exigées, et finallement, on termine par le façonage et le calibrage de la plaque.

2. Procédé selon la revendication 1, **caractérisé en ce que** le décor est crée par la fixation sur le côté derrière de la plaque, d'une feuille imprimée d'un systém des éléments décoratifs.

3. Procédé selon l'une quelconque des revendications précédentes, **caractérisé en ce que** le systém des élements décoratifs opaques ou de la transparence réduite est determiné par la vérification des écarts de l'effect lumineux du projet de base de l'arrangement desdits éléments par rapport à l'effect lumineux résultant et ensuite par la correction des écarts en changeant du moins de l'un des paramètres du moins de l'un segment sur l'un des côtés de la plaque, lesdits paramètres renfermant le nombre, grandeur et densité des caractères et des fentes, l'orientation du segment et la variante de couleurs.

4. Procédé selon l'une quelconque des revendications précédentes, **caractérisé en ce que** des éléments décoratifs sont produits en appliquant le colorant apte à être traité à chaud, ledit colorant est appliqué par la technique telle que l'impression, vernissage, remplissage des fentes ou sous forme de décalque.

5. Procédé selon l'une quelconque des revendications 1 à 3, **caractérisé en ce que** des éléments décoratifs sont produits en remplissant des creux, formés par le laminage ou la taillerie, par le colorant apte à être traité à chaud.

6. Procédé selon des revendications 1 à 3, **caractérisé en ce que** l'on utilise les colorants apte à être traité à chaud, par exemple couleur vitrifiable, céramique, métallique ou l'émail.

7. Procédé selon l'une quelconque des revendications 1 à 5, **caractérisé en ce que** l'on utilise les colorants qui ne sont pas apte à être traité à chaud, par exemple les colorants sur la base de la résine, des émails, UV ou les colorants durcis chimiquement.

8. Procédé selon l'une quelconque des revendications précédentes, **caractérisé en ce que** le colorant décoratif utilisé est traité par cuisson ou séchage ou durcissement en vue de l'obtention des propriétés mécaniques spécifiques.
